

## UNITED STATES PATENT OFFICE

VICTOR SCHOLZ, OF LEIPZIG, GERMANY, ASSIGNOR TO THE FIRM ATLAS AGO  
CHEMISCHE FABRIK, OF MOLKA, NEAR LEIPZIG, GERMANY

## PROCESS OF PREPARING LINOXYN OR MATERIALS SIMILAR TO LINOXYN

No Drawing. Application filed March 21, 1929, Serial No. 348,974, and in Germany December 21, 1925.

For the manufacture of linoleum linoxyn is used as a starting body for producing the linoleum cement.

Linoxyn is a consistent polymerized and oxidized linseed-oil the iodine number of which decreases through the process of polymerization and oxidation from 186 to about 50-60.

In the manufacture of linoleum Walton 10 linoxyn is used the most, being prepared by thin oil varnish trickling over cloth in oxidizing-houses in temperatures from 40-60° C., so that through flooding the cloth several 15 times daily for six months, a layer of linoxyn is obtained of about 2 cm. thickness. Because of the inconvenience of this Walton process, efforts have been frequently made to produce linoxyn by a quick-oxidation process, of which the Taylor process is the most 20 important. In this latter process heated oil-varnish is blown with air into drum-shaped vessels provided with an agitator which begins to act as soon as the oil, getting thicker and thicker, commences to resist the passage 25 of air. Taylor linoxyn is a yellow-brown elastic body which does not attain the quality of the Walton linoxyn. In Taylor linoxyn the glycerine group of the linseed-oil is destroyed and is lost in the waste-gases such as 30 acrylic acid or similar inferior acids. Taylor linoxyn is not oxidized through so much and melts easier than Walton linoxyn the high fusing point of which renders it preferable for the manufacture of linoleum.

35 It has now been found that excellent linoxyns with high melting points can be produced in a surprisingly simple manner out of varnishes as well as out of pure linseed oils and that the catalyst (lead, manganese, 40 nickel, cobalt, zinc, tin, cadmium, &c., or the oxides of these, or resinate or linoleate compounds) merely affects the proportions of solubility of the linoxyns obtained and their melting-points.

45  $\frac{1}{2}\%-2\%$  of catalyst, e. g. litharge or linoleate of lead, is dissolved being stirred at a moderate temperature of 120-250° C. in linseed oil, whereupon it is worked into linoxyn in two stages the first one of which is known 50 in itself.

First stage: In heatable and coolable, tiltable dishes, troughs, or vessels with outlet-hood and with or without agitator, pure linseed oil or linseed oil plus  $\frac{1}{2}\%-2\%$  of catalyst, e. g. 2% of litharge, is blown at a possibly low temperature (60-150° C.) with cold or warm air, and during the blowing process the oil-temperature is kept at the same height if possible, e. g. at 100° C. Thus a glassy, tenacious, yellow-brown, lustrous, viscous, 60 body is formed, which finally tears off from the boiler-wall, copper and agitator, entirely stopping the passage of air or permitting it only in the way of occasional head-sized bubbles and with an iodine number of about half 65 that of the linseed oil iodine number, i. e. from 90-95 instead of 186. An increase of temperature leads at best to darker smearable products, but no further oxidation takes place. The limit of oxidation of the linseed oil or 70 the like oils with saturated groups is attained by the blowing process.

It was then found that these blown linseed oils or half oxidized linoxyns of the Taylor linoxyn kind can be further oxidized and improved in a surprisingly simple manner by 75 means of a second process.

This second process consists simply in the blown, tenacious, viscous, lustrous, yellow-brown products being kneaded in heatable 80 and coolable, high-shovelled kneading machines with access of air, the process, as regards duration and final product, depending merely on the temperature at which the kneading takes place.

The kneading shovels force and press air into the kneaded mass oxidizing the same more and more, the blown product losing its lustre, getting dull, becoming lighter in color and turning gradually from yellow-brown 90 into a yellow-orange up to yellow-white, according to the kind of catalyst, and finally dropping into fine loose little crumbs while pungent waste-gases are developing. A tenacious blown oil for example made with 95 2% of litharge, of yellow-brown color, changes during a three or four hours' kneading process at 100° C. into a fine-crumb light-yellow-orange colored linoxyn, while blown oils prepared with other catalysts or pure 100

blown linseed oil, will finally yield yellow to yellow-white crumbly to powdery linoxyns.

If the kneading process is carried on too long or at too high a temperature, many pungent vapours of inferior acids which very much irritate the eyes are developed, the product becoming almost white, very hot and powdery, and if the cooling and spreading does not take place quickly, it will carbonize in itself while developing heat.

The kneading of air into blown oil or blown varnish is accomplished slowly even in the cold, i. e. in cold, unheated kneading machines, a slight heat developing by itself. Through the heating and cooling arrangement of the kneading machine the conduct of the process can be easily controlled and interrupted when the kneaded linoxyn has assumed the quality which experience has proved to be the most favorable. The kneading process is generally interrupted when the linoxyn has become light-colored and of a fine crumb and when pungent vapors are developing, and in order to stop further self-oxidation, cooling and spreading of the kneaded linoxyn must take place immediately.

In order to prevent the development of decomposing gases and products during the kneading process, which gases are mostly of an acidic nature, small quantities of from  $\frac{1}{2}\%$  to 2% of chemical bases may be added to the blowing or kneading oils and oil-mixtures, and it has been found that for this purpose organic bases are especially suitable, e. g. such as amides and amines ( $\text{NH}_2$  or  $\text{NH}_3$ ), group-containing bodies such as aniline oil, naphthylamine, urea, or similar bodies.

According to the catalyst used, or even without the use of a catalyst in the blowing process, the ready kneaded linoxyn can be adapted in its qualities, especially as regards its melting point and its solubility, to the different purposes.

Kneaded linoxyn can be worked up in the usual manner or directly in the kneading machine after being finished with resins or copals to linoleum cement. All that is necessary for this purpose is: to add to the linoxyn produced in the kneading machine and having become finely crumbed, resin and kauri-copal in the proportion of 5 resin and 3 kauri-copal to 25 linoxyn, the resin and copal being powdered and melted for the direct production of linoleum cement which can then be transferred in the known manner with color, wood-meal and cork-meal in proportion of 33 parts of linoleum cement to 66 parts of pigments and filling substances, into linoleum ground-mass and thus into linoleum.

Besides linseed oil, other oils containing unsaturated groups can be worked in the same way into tenacious, linoxynlike, poly-

merized and oxidized bodies, e. g. wood-oil, Hevea-oil, Perilla-oil, sunflower-oil, nut-oil, hemp-oil or mixtures of these with each other or with linseed oil. Finally non-drying oils of the oxy-oleic acid series containing unsaturated groups such as castor-oil by itself or mixed with linseed-oil and similar drying oils, can be blown together and kneaded and transferred into firm-crumbly end-products, which are again of variable qualities according to the choice of mixed oils and catalysts. In this way linoxyns and linoleum-cements of any required elasticity can be produced by the addition of non-drying oils with unsaturated groups, e. g. castor-oil, to the saturated drying-oils during the blowing- and kneading-processes.

According to whether the unmixed or mixed oils are blown or kneaded, or whether a catalyst is introduced into the oils before blowing and kneading or during these processes, the end-product can be regulated with regard to cold-resistance, fusibility and solubility in different solvents.

Finally, linoxyns can be used also for the manufacture of soaps, for the steeping of canvas, tilts, horse-blankets, knapsacks, umbrellas, &c. For these purposes the linoxyns prepared according to this invention are saponified with alkalies, the soap-solution being eventually mixed or emulsified with tallow wax, glue- or leather-solution or other additions, and on the materials impregnated with the linoxyn soap the insoluble oxy-soap is precipitated with baths of watery sulphate or acetate of alumina, which renders the textures waterproof, preserves their full porosity and imparts a velvety touch to them.

Linoxyns, especially those made of sebacic acid, mixed with soda, borax or the like saponifying materials dissolved in boiling water, may be used also as bleaching and washing materials, because during the saponification the peroxide groups of the linoxyns give off oxygen.

While I have described the use of air in treating the oils, it is obvious that the resulting oxidation is produced by the oxygen content of the air and I therefore claim in some of my claims broadly the use of oxygen.

#### Claims:

1. A substance which consists of a polymerized and oxidized oil of the type having a molecule with an unsaturated group and which has a fine-crumbly, flaky yellowish opaque consistency as a result of a kneading process to which said oil has been subjected after a preparatory conversion into a jelly by oxidation effected by air blown through the oil at an elevated temperature.

2. The process of manufacturing a linoxyn-like material comprising blowing oxygen through an oil, the molecules of which have unsaturated groups, until it is con-

verted into a viscous body and then kneading oxygen into said viscous body until it attains a fine, crumby, opaque consistency.

3. The process of manufacturing linoxyn  
8 which comprises blowing oxygen through linseed oil until the latter is converted into a viscous body and subsequently kneading oxygen into said viscous body until it attains a fine, crumby, opaque consistency.

13 4. In the process claimed in claim 2, adding a catalyst to the oil before blowing oxygen therethrough.

15 5. In the process of claim 2 adding a basic material before commencing the kneading 16 operation in quantities sufficient to prevent the development of acid gases.

6. In the process claimed in claim 2 rapidly cooling the product after it has attained a fine, crumby, opaque consistency to prevent 20 continued oxidation and the development of acid gases.

7. The process of manufacturing linoxyn  
25 which consists in adding a catalytic compound to linseed oil, blowing air heated to 100° C. through the resulting mixture until the oil has been converted into a viscous body, kneading the air into said viscous body while maintaining the temperature of the latter at about 100° C. until it attains a fine, crumby, 30 opaque consistency and then rapidly cooling the material to avoid self-oxidation thereof and the development of acid gases.

In testimony whereof I have signed my name to this specification.

35 VICTOR SCHOLZ.

verted into a viscous body and then kneading oxygen into said viscous body until it attains a fine, crumby, opaque consistency.

3. The process of manufacturing linoxyn which comprises blowing oxygen through linseed oil until the latter is converted into a viscous body and subsequently kneading oxygen into said viscous body until it attains a fine, crumby, opaque consistency.

13 4. In the process claimed in claim 2, adding a catalyzer to the oil before blowing oxygen therethrough.

5. In the process of claim 2 adding a basic material before commencing the kneading 15 operation in quantities sufficient to prevent the development of acid gases.

6. In the process claimed in claim 2 rapidly cooling the product after it has attained a fine, crumby, opaque consistency to prevent 20 continued oxidation and the development of acid gases.

7. The process of manufacturing linoxyn which consists in adding a catalytic compound to linseed oil, blowing air heated to 25 100° C. through the resulting mixture until the oil has been converted into a viscous body, kneading the air into said viscous body while maintaining the temperature of the latter at about 100° C. until it attains a fine, crumby, 30 opaque consistency and then rapidly cooling the material to avoid self-oxidation thereof and the development of acid gases.

In testimony whereof I have signed my name to this specification.

35 VICTOR SCHOLZ.

#### CERTIFICATE OF CORRECTION.

Patent No. 1,794,325.

Granted February 24, 1931, to

VICTOR SCHOLZ.

It is hereby certified that the above numbered patent was erroneously issued to the firm "Atlas Ago Chemische Fabrik", as assignee of the entire interest in said invention, whereas said patent should have been issued to the inventor, said Scholz and to the firm Atlas Ago Chemische Fabrik, said firm being assignee of one-half interest only in said invention, as shown by the records of assignments in this office; and that the said Letters Patent should be read with this correction therein that the same may conform to the record of the case in the Patent Office.

Signed and sealed this 29th day of September, A. D. 1931.

(Seal)

M. J. Moore,  
Acting Commissioner of Patents.

**CERTIFICATE OF CORRECTION.**

Patent No. 1,794,325.

Granted February 24, 1931, to

**VICTOR SCHOLZ.**

It is hereby certified that the above numbered patent was erroneously issued to the firm "Atlas Ago Chemische Fabrik", as assignee of the entire interest in said invention, whereas said patent should have been issued to the inventor, said Scholz and to the firm Atlas Ago Chemische Fabrik, said firm being assignee of one-half interest only in said invention, as shown by the records of assignments in this office; and that the said Letters Patent should be read with this correction therein that the same may conform to the record of the case in the Patent Office.

Signed and sealed this 29th day of September, A. D. 1931.

(Seal)

**M. J. Moore,  
Acting Commissioner of Patents.**